

## UNITED STATES PATENT OFFICE

2,371,102

## DIQUINONYL AMIDES IN VAT COLOR COMPOSITIONS

Roy Herman Kienle and Chester Albert Amick,  
Bound Brook, N. J., assignors to American Cyanamid Company, New York, N. Y., a corporation of Maine

No Drawing. Application July 1, 1943,  
Serial No. 493,134

10 Claims. (Cl. 8—70)

This invention relates to a new type of dyeing and printing assistant, dye compositions containing these assistants and products printed therefrom.

Use of printing-color pastes containing dyes, particularly in printing operations using vat dyes, is sufficiently well-known so that the procedure has become almost standardized. The actual color source may be either a dye paste or a dye powder. In addition to the real color, a dye paste usually contains agents to prevent drying-out, settling and/or freezing. Dye powders, not being subject to these difficulties, do not require these agents but they usually contain agents or are so processed as to promote dispersibility.

In either case, the dye paste or dye powder must be admixed with suitable thickener, usually a gum dispersion, to form a printing-color paste which is suitable for application. In the case of vat dyes, it is also necessary to add a reducing agent and usually an alkali. Because the color yield from printing-color pastes often decreases rapidly as the paste ages after being made up, these printing-color pastes are usually prepared by the fabric finishers just before they are to be used.

The printing-color pastes, however compounded, are then applied to textile, paper or other fabric materials for decorative or protective purposes. The printed pieces are dried, aged in a steam ager, treated with an oxidizing agent, rinsed and finally dried. Usually in processing textiles, the printed fabric also is soaped at or near the boil with about a 0.1% soap solution and again rinsed before the final drying operation.

In making up and applying printing-color pastes it has been found that a material suitable for use as a printing assistant is of advantage in obtaining maximum color yield. The exact way in which these materials act to produce an improved color yield in printing is not entirely understood. It is with these printing aids or assistants that the present invention is particularly concerned.

Although printing aids are desirable in the printing-color pastes, the exact point at which they are added may vary. Dye pastes may contain printing aids as one of their components and printing-color pastes made therefrom will obviously contain the printing assistant. Where a printing assistant is not present in the dye paste, it may be added at the time of making up the printing-color paste.

It is preferable, however, that the printing assistant be incorporated in the actual dye paste. Their addition at the proper point in the manu-

facture of the paste is not only easier, but in addition they are thus generally more uniformly dispersed throughout a printing-color paste made therefrom. As a result, the printing assistants usually operate more effectively when the printing-color paste is finally applied to the fabric.

It is only relatively recently that dye powders suitable for use in making up printing-color pastes have been available. Most of the printing aids previously used in dye pastes, being either liquid in form or extremely hydroscopic, can not be used with dye powders, the latter being necessarily limited to the use of dry solids. Nevertheless, it is desirable that printing assistants be incorporated in the powders at the time of manufacture for the same reasons which apply in the case of dye pastes.

Dye pastes containing various liquid printing assistants have been made. Among the liquid materials used are the alkylol amines, for example, triethanol amine; and/or polyhydric alcohols such as glycerine, glycol, diethylene glycol and the like. Various derivatives therefrom also have been tried. If a printing aid is to be incorporated in a dye powder, a solid printing aid is necessary. Examples of such solids which have been used in the past include the hydrochlorides of alkylol amines; silver salt (sodium anthraquinone beta-sulfonate); anthraquinone and certain metal salts such as those of cobalt and iron.

Unfortunately, most of these printing aids previously used are not as satisfactory as may be desired. Many of them will not in all cases produce the intensification of color for which they were intended. Others, such as the polyhydric alcohols, cause deterioration of the printing-color pastes so that marked variations in the strength of prints therefrom are observable even after the printing-color paste has been allowed to stand for only a relatively short time. Many of them are satisfactory with some colors but have an adverse effect on others, even to the extent of visibly altering the shade. None of them are suitable without modification for use both in paste and powder compositions.

There remains, therefore, a demand for suitable printing assistants which will produce a satisfactory color intensification and will not cause deterioration of the dyeing or printing composition on standing. Preferably also, the assistants should be useful both with dye pastes and dye powders and in addition should be readily available or cheaply and easily prepared. It is, therefore, the object of the present invention to pro-

vide a new type of printing assistant which possesses these desirable properties.

In general, the object of the present invention is accomplished by making use of one or more of the diquinonyl carboxylic acid diamides as printing assistants. These compounds may be generically represented by the type formula



in which Ac represents the residue of a cyclic or aliphatic dibasic acid, and Q and Q' represent quinonyl groups such as those derived from naphthoquinone and anthraquinone. Typical of the diamides of the present invention is N,N'-di-(alpha-anthraquinonyl) fumaric acid diamide, which has the probable formula



So far as the present invention is concerned, the assistants may be added to the printing-color pastes at any point in the preparation of the latter. They may be incorporated into the thickener; into the dye pastes or powders or may be blended directly into the printing-color paste. However, as pointed out above, it is preferable that they be incorporated in the dye paste or powder during manufacture.

The use of this new class of printing assistants possesses a number of important advantages. These compounds are dry solids, which may be readily powdered and blended in dye powders and are soluble or dispersible in dye paste suspensions. They have, therefore a general application in both dye pastes and dye powders. They do not cause deterioration of printing-color pastes on standing. They encourage the production of excellent color yields even under hot ageing conditions. Their use is simple since they may be employed as powders or as suspensions in water or alcohol, producing excellent color yields whatever the mode of admixture.

In preparing the compounds to be used as the printing assistants of the present invention the dicarboxylic acid may be quite widely varied. The compounds may be derived from either cyclic or aliphatic dicarboxylic acids. Of the cyclic dicarboxylic acids, phthalic acid is perhaps the most common and its derivatives have been found to give good results when used according to the present process. The invention however is not meant to be so limited but includes, for example, derivatives of isophthalic, terephthalic, polyhydrophthalic acids, the endoalkylenepolyhydrophthalic acids such as endomethylene tetrahydrophthalic and endoethylene hexahydrophthalic acids and the like, and the naphthalic acids, as well as substituted acids derived therefrom.

Where derivatives of aliphatic carboxylic acids are used, the original acid or anhydride may be varied over a considerable range. If the original acid is considered to have the formula



in the case of the anhydride, C<sub>y</sub> in the generic formula may vary over the range of y=0 in the case of oxalic acid to about y=8 without departing from the scope of the present invention. However, where y is greater than about 6, trouble is encountered in preparing the derivatives. Above about y=8, there is a tendency for the compounds to become sufficiently water insoluble to prevent satisfactory use. The acids may be either saturated acids such as malonic, succinic, glutaric, adipic, sebacic and the like or unsaturated such as maleic, fumaric and the like.

As pointed out in connection with the generic formula, Q and Q' represent quinonyl groups such as those of the naphthoquinones and anthraquinones. Paraquinonyl derivatives such as those from alpha-naphthoquinone and p-anthraquinone were found to give particularly good results according to the present invention. The invention however is not necessarily so limited. Similarly good results were obtained for example from the derivatives of beta-naphthoquinone and beta-anthraquinone. While the theoretical possibilities do not require that Q and Q' be the same quinonoid radicals, practically the present invention is so limited. Similar compounds in which Q and Q' are not identical are considered in our copending applications for U. S. Letters Patent, Serial Nos. 493,135-6, filed of even date.

While the dye and printing-color paste compositions of the present invention are not limited to the use of any particular dyes or dye forms, they are especially suitable for use with vat-dyes in either paste or powder form. Particularly good results may be obtained using the vat-dye powders of high autodispersibility set forth in Crossley et al., United States Reissue Patent No. 21,402, reissued March 19, 1940. By combining the color materials of that patent into printing paste compositions containing the assistants of the present invention, the full advantages of both may be gained with a resultant simplicity in use, excellence of shade and sharpness of color.

Printing pastes made in this way have the particular advantage that the dyes remain in a highly dispersed state as individual particles rather than as dispersions of particle aggregates. In the present specification and claims, where highly-dispersed dyes are referred to, reference to pastes in which the dye particles are so dispersed is intended.

The invention will be more fully set forth in connection with the following examples which are intended to be illustrative and not by way of limitation. All parts are by weight unless otherwise noted.

In the succeeding examples, test prints were made on two different fabrics. Where rayon is referred to, a titanium-dioxide-pigmented, all-viscose-rayon flat crepe was used. The cotton fabric referred to is an 80 x 80 bleached, unmercerized, cotton print-cloth. Ageing of the prints was carried out in a steam ager which was constructed in such a manner that controlled temperatures could be used. The temperature range normally used was 100°-105° C. Those ageing referred to as plant or hot ageing were carried out in the temperature range of about 106°-110° C. In the case of the cotton prints ageing periods of 3 minutes, 5 minutes or both

were used. The shortest period which gives a satisfactory ageing is preferable.

*Example 1*

A paste was prepared by slurring 2,000 parts of 177 British gum (Stein-Hall) in 5,000 parts of water and the mixture was heated with continuous stirring until the temperature reached about 185° F. Heating was continued for about 1½ hours after which 450 parts of powdered potassium carbonate and 450 parts of powdered sodium carbonate were added and the mixture stirred until the carbonates dissolved. Heating was discontinued but stirring was continued until the temperature reached approximately 150° F. at which time 700 parts of sodium sulfoxylate were dissolved therein, 600 parts of glycerine were added and the paste bulked to about 10,000 parts. Stirring was continued until the paste cooled to room temperature. In the succeeding examples this paste is referred to as thickener A.

*Example 2*

720 parts of B-2 British gum and 720 parts of KAC-4 gum (Stein Hall) were added to 5,600 parts of water and heated over a steam bath for approximately 1½ hours after the temperature reached 185°-190° F. The source of heat was then removed but stirring was continued until the temperature decreased to 120° F. at which time 1,200 parts of potassium carbonate which had been previously dissolved in 1,000 parts of water was added to the cooked gum. 1,560 parts of sodium sulfoxylate formaldehyde were dissolved in 1,500 parts of water at a temperature of about 140° F. and added to the common mixture with stirring until the whole was thoroughly mixed. Finally, 360 parts of glycerine were added and after thorough stirring the whole was bulked to 12,000 parts. In the succeeding examples this mixture is referred to as thickener B.

*Example 3*

6 parts of a dispersible Orange R powder (C. I.—1217), prepared according to U. S. Reissue Patent 21,402 and containing about 2.4 parts of real dye, were pasted with 3 parts of water and 91 parts of thickener A. This was used as the control sample. 20 parts of N,N' di(beta-anthraquinonyl) fumaric acid amide were slurred with 80 parts of water and ground in a ball mill until a uniform suspension was obtained. 3 parts of this suspension were then added to 6 parts of the Orange R powder together with 91 parts of thickener A. Each of these pastes were printed on rayon and cotton. The printed pieces were air dried, and aged in a steam ager. After ageing the pieces were oxidized, rinsed, soaped in a 1% soap solution for 5 minutes at the boil, again rinsed and ironed dry. The prints made from the paste containing the N,N' di(beta-anthraquinonyl) amide gave much stronger color yields than those made from the paste in which no printing assistant was used.

*Example 4*

The procedure of Example 3 was repeated except that 3 parts of a 20% suspension of N,N' di(alpha-anthraquinonyl) fumaric acid amide were used instead of the beta product of Example 3. The prints made from the paste containing the printing assistant were smoother, brighter and appreciably stronger than those made from the paste containing water only.

5 The procedure of Example 3 was duplicated exactly except that a 3% suspension of N,N' di(alpha-anthraquinonyl) maleic acid amide was used. Again the prints obtained from the paste containing the amide of maleic acid were much stronger both on rayon and cotton pieces than those obtained from the control sample.

10

*Example 6*

15 The procedure of Example 3 was duplicated except that a 3% suspension of N,N' di(beta-anthraquinonyl) maleic acid amide was used. Prints obtained from the paste containing the amide of maleic acid were much stronger, smoother and brighter.

15

*Example 7*

20 The procedure of Example 3 was followed except that the di-anthraquinonyl amide of fumaric acid was replaced by the di-anthraquinonyl amide of phthalic acid. Both the di-alpha or the di-beta compound were used. Prints made from pastes containing both the di-alpha and the di-beta anthraquinonyl amides of phthalic acid were definitely superior to those obtained from the control sample.

25

*Example 8*

25 The procedure of Example 3 was repeated exactly except that the fumaric acid amide was replaced by N,N' di(anthraquinonyl) succinamide. In this case also, both the beta and the alpha compound were used. Prints obtained from the pastes containing the di-anthraquinonyl amides gave much stronger color yields than those made from the pastes containing water only. These assistants had the property of reducing the length of time that was necessary to develop the maximum color value during the ageing operation. This is a distinct advantage because it permits a speed-up in the ageing operation, an important commercial consideration.

30

*Example 9*

30 6 parts of the alpha-anthraquinonyl diamide of fumaric acid were slurred in 94 parts of water and then milled in a ball mill for 18 hours. 5 parts of Golden Orange G powder (C. I.—1096), 55 prepared according to U. S. Reissue Patent 21,402 and containing about 1 part of real dye were slurred with 5 parts of the 6% suspension of the alpha-anthraquinonyl diamide of fumaric acid. After the mixture was intimately mixed, 90 parts of thickener B were added. 5 parts of Golden Orange G were then slurred with 5 parts of water and 90 parts of thickener B to provide a control sample. Each of the pastes were printed on rayon. The printed pieces were then air-dried, aged, oxidized, rinsed, soaped in 1% soap solution for 5 minutes at the boil, then rinsed and ironed dry. The prints obtained from the paste containing the alpha-anthraquinonyl diamide of fumaric acid were stronger and brighter than those obtained from the control. This was particularly noticeable when aged under practical mill conditions.

35

*Example 10*

70 75 A sample of wet presscake of Orange R, (C. I.—1217) was dispersed with the sodium salt of disulfodinaphthyl methane and adjusted with water to contain about 12% real dye. 10 parts of this slurry were mixed with the printing assistant used in Example 9. Then to this mixture was added 85

parts of thickener B and the whole was thoroughly mixed. A second 10 parts of the Orange R was likewise mixed with 5 parts of water and 85 parts of thickener B. Prints made from the paste containing the printing assistant were much stronger both on cotton and rayon than those obtained from the paste containing water only.

*Example 11*

10 parts of Dark Blue BO dispersed powder, (C. I.—1099) prepared according to U. S. Reissue Patent 21,402 and containing about 3.7% real dye were dry blended with 0.3 parts of N,N' di(alpha-anthraquinonyl) fumaramide. To this mixture, 90 parts of thickener B were added and after intimate mixing prints were made of this paste on cotton and rayon. A second 10 parts of the Dark Blue BO were then mixed with thickener B without any printing assistant being added. This was the control sample. This paste was also printed on cotton and rayon. The prints obtained from the paste containing the printing assistant were definitely stronger and brighter than those obtained from the control sample. Again this was especially noticeable when plant ageing conditions were simulated.

*Example 12*

The procedure of Example 10 was followed except that the diamide of fumaric acid was replaced by the reaction product of 2-amino-alpha-naphthoquinone and maleic acid and of 5-amino-alpha-naphthoquinone and maleic acid. The prints obtained from the pastes containing the printing assistants were much stronger than those obtained from the paste containing water only.

We claim:

1. A color composition comprising a vat dye and a dicarboxylic acid diamide represented by the formula



in which Ac represents the residue of a dicarboxylic acid selected from the group consisting of the saturated and unsaturated aliphatic dicarboxylic acids of from 2-10 carbon atoms, the phthalic acids, the naphthalic acids, the polyhydrophthalic and naphthalic acids and the alkyl-substituted phthalic and naphthalic acids, and Q and Q' represent the same quinonyl radicals selected from the group consisting of the naphthoquinonyl and anthraquinonyl radicals.

2. A dye powder composition comprising a vat dye and a powdered dicarboxylic acid diamide represented by the formula



in which Ac represents the residue of a dicarboxylic acid selected from the group consisting of the saturated and unsaturated aliphatic dicarboxylic acids of from 2-10 carbon atoms, the phthalic acids, the naphthalic acids, the polyhydrophthalic and naphthalic acids and the alkyl-substituted phthalic and naphthalic acids, and Q and Q' represent the same quinonyl radicals selected from the group consisting of the naphthoquinonyl and anthraquinonyl radicals.

3. A dye composition comprising a vat dye powder of high autodispersibility, and a powdered dicarboxylic acid diamide represented by the general formula



in which Ac represents the residue of a dicarboxylic acid selected from the group consisting of the saturated and unsaturated aliphatic dicarboxylic acids of from 2-10 carbon atoms, the phthalic

acids, the naphthalic acids, the polyhydrophthalic and naphthalic acids and the alkyl-substituted phthalic and naphthalic acids, and Q and Q' represent the same quinonyl radicals selected from the group consisting of the naphthoquinonyl and anthraquinonyl radicals.

4. A color composition according to claim 1 in which Q and Q' represent a naphthoquinonyl group.

10 5. A color composition according to claim 1 in which Q and Q' represent an anthraquinonyl group.

6. A printing paste composition comprising a vat dye, a thickener and a dicarboxylic acid 15 diamide represented by the general formula



in which Ac represents the residue of a dicarboxylic acid selected from the group consisting of the 20 saturated and unsaturated aliphatic dicarboxylic acids of from 2-10 carbon atoms, the phthalic acids, the naphthalic acids, the polyhydrophthalic and naphthalic acids and the alkyl-substituted phthalic and naphthalic acids, and Q and Q' represent the same quinonyl radicals selected from the group consisting of the naphthoquinonyl and 25 anthraquinonyl radicals.

7. A printing paste composition comprising a thio-indigo vat dye, a thickener and a dicarboxylic acid diamide represented by the general formula



in which Ac represents the residue of a dicarboxylic acid selected from the group consisting of the 30 saturated and unsaturated aliphatic dicarboxylic acids of from 2-10 carbon atoms, the phthalic acids, the naphthalic acids, the polyhydrophthalic and naphthalic acids and the alkyl-substituted phthalic and naphthalic acids, and Q and Q' represent the same quinonyl radicals selected from the group consisting of the naphthoquinonyl and 35 anthraquinonyl radicals.

40 8. A printing paste composition comprising a highly-dispersed thio-indigo vat dye, a thickener and a dicarboxylic acid diamide represented by the general formula



in which Ac represents the residue of a dicarboxylic acid selected from the group consisting of the 50 saturated and unsaturated aliphatic dicarboxylic acids of from 2-10 carbon atoms, the phthalic acids, the naphthalic acids, the polyhydrophthalic and naphthalic acids and the alkyl-substituted phthalic and naphthalic acids, and Q and Q' represent the same quinonyl radical selected from the group consisting of the naphthoquinonyl and 55 anthraquinonyl radicals obtainable by compounding a collodized vat dye powder of high autodispersibility and the dicarboxylic acid diamide with the thickener.

60 9. A method of printing with vat colors which comprises printing a fabric with a printing paste composition comprising a vat dye, a thickener and a dicarboxylic acid diamide represented by the general formula



in which Ac represents the residue of a dicarboxylic acid selected from the group consisting of the 70 saturated and unsaturated aliphatic dicarboxylic acids of from 2-10 carbon atoms, the phthalic acids, the naphthalic acids, the polyhydrophthalic and naphthalic acids and the alkyl-substituted phthalic and naphthalic acids, and Q and Q' represent the same quinonyl radicals selected from the group consisting of the naphthoquinonyl and anthraquinonyl radicals.

represent the same quinonyl radicals selected from the group consisting of the naphthoquinonyl and anthraquinonyl radicals.

10. An article of manufacture comprising a fabric printed with a composition comprising a <sup>5</sup> vat dye and a dicarboxylic acid diamide represented by the general formula



in which Ac represents the residue of a dicarboxylic acid selected from the group consisting of the

saturated and unsaturated aliphatic dicarboxylic acids of from 2-10 carbon atoms, the phthalic acids, the naphthalic acids, the polyhydrophthalic and naphthalic acids and the alkyl-substituted phthalic and naphthalic acids, and Q and Q' represent the same quinonyl radicals selected from the group consisting of the naphthoquinonyl and anthraquinonyl radicals.

ROY HERMAN KIENLE.  
CHESTER ALBERT AMICK.

CERTIFICATE OF CORRECTION.

Patent No. 2,371,102.

March 6, 1945.

ROY HERMAN KIENLE, ET AL.

It is hereby certified that error appears in the printed specification of the above numbered patent requiring correction as follows: Page 1, first column, line 18, for "dispension" read --dispersion--; and that the said Letters Patent should be read with this correction therein that the same may conform to the record of the case in the Patent Office.

Signed and sealed this 14th day of August, A. D. 1945.

Leslie Frazer

(Seal)

First Assistant Commissioner of Patents.